

# UNITED STATES PATENT OFFICE.

MARK GARTERED RAY, OF PERTH AMBOY, NEW JERSEY.

## FIRE AND WATER PROOF BUILDING MATERIAL.

No. 885,376.

Specification of Letters Patent.

Patented April 21, 1908.

Application filed December 28, 1907. Serial No. 408,372.

To all whom it may concern:

Be it known that I, MARK GARTERED RAY, a citizen of the United States, residing at Perth Amboy, in the county of Middlesex and State of New Jersey, have invented new and useful Improvements in Fire and Water Proof Building Material, of which the following is a specification.

This invention relates to composite building material, and it has for its object to produce a fire proof and water proof material which may be used in sheet or broad board form, as a substitute for lath and plastering, and for other purposes.

To this end my invention consists in the combination and union of ingredients forming fire and water proof building material as hereinafter more fully described and particularly set forth in the claim.

To make boards according to my invention to serve as a substitute for lath and plaster, I take first, a sheet of soft, unsized paper board of convenient width and length to be easily handled, say wide enough to extend from center to center of the first and third studs and overlapping one stud midway, and in length anywhere from three feet to the height of the room, and lay this sheet upon a table and coat it heavily with hot glue. On that I place a sheet of asbestos; on that another coat of glue; on that another sheet of soft paper board, and so on until the desired thickness is attained. Then I place this slab of sheets and glue under a heavy

press and let it remain until it is dry enough for the glue to become set. To obtain a glue which is impervious to water I use a gum that is soluble only in strong spirit, preferably shellac dissolved in alcohol to the consistency of thick varnish. This constitutes a very strong glue but it has not sufficient affinity for either the asbestos or the pulp of the paper board to penetrate them much yet, a sizing having a watery menstruum readily saturates them. I therefore prepare first, a thin

paste of some adhesive substance such as common flour or animal glue in water, and mix it in about equal proportions with the dissolved shellac, hot, and immediately ap-

ply it as the glue between the boards, above referred to. This watery paste performs the double office of holding the shellac in solution during the time required to apply it, even though the alcohol which dissolved it becomes evaporated by the heat; and of readily permeating the porous boards and carrying with it the shellac, thus entirely closing the pores of the individual boards, and, under the pressure applied, uniting the whole mass as a single board impervious to water.

This composite board has some elasticity; is extremely strong; cannot be split and does not flake off when nails are driven through it. It may be sawed, planed, or turned in a lathe like very close grained wood, and is susceptible to a high polish. In its plastic condition, when piled up as a slab, it may be pressed into molds for ornamental purposes and worked much like sheet metal. As a substitute for lath and plaster it may be immediately covered with wall paper; no need of waiting for it to dry. By filling the line joints with the glue described, and sand papering the lines, a surface as smooth as calamine may be provided for painting or other decoration. Being firmly nailed to the house timbers this boarding cannot be jarred off, and water from leaky roofs will not injure it. The asbestos in it is particularly designed to prevent or to stop the spreading of fires.

So far as my experiments have extended I find shellac to be the best gum to use for the glue, but any of the resinous gums which are insoluble in water and require strong spirit as a solvent, may be used; and I may use as a leader to this gum, any starchy or glutinous substance that is readily soluble in water, provided its nature and proportions are such that its union under pressure with the gum used renders it impervious to water.

Having thus fully described my invention, what I believe to be new and desire to secure by Letters Patent is the following:

1. In building material, the combination of one or more sheets of soft paper board, with one or more sheets of asbestos, and a

glue uniting them; the said glue comprising gum shellac dissolved in alcohol, and a paste having water as a menstruum.

2. A building material comprising one or 5 more sheets of soft paper board, one or more sheets of asbestos and a glue uniting them; the glue comprising a resinous gum dissolved in spirits and insoluble in water, and a leader

consisting of a starchy or glutinous substance dissolved in water, all combined as described. 10

In testimony whereof I affix my signature, in presence of two subscribing witnesses.

MARK GARTERED RAY.

Witnesses:

S. R. FARRINGTON,  
TULU DIMOND.